

## I

3,069,256

## PREPARATION OF THORIUM INTERMETALLIC COMPOUND DISPERSION

Robert J. Teitel and George B. Cobel, Midland, Mich., assignors to The Dow Chemical Company, Midland, Mich., a corporation of Delaware

No Drawing. Filed Aug. 17, 1960, Ser. No. 50,095

4 Claims. (Cl. 75—122.7)

The invention relates to a method of preparing a dispersion of thorium bismuthide or thorium-lead compound in bismuth lead or bismuth-lead alloy and more particularly relates to a method of preparing a dispersion of such a thorium intermetallic compound in fine particulate form.

In nuclear reactors neutrons escaping from the core are often utilized to breed, or form, additional fuel material. Breeding consists mainly of exposing a blanket material such as thorium to the escaping neutrons. Very fine dispersions of thorium bismuthide in bismuth or bismuth-lead alloy or thorium-lead compound in lead or lead-bismuth alloy are an advantageous form of thorium which is useful as a fluid blanket material.

A desirable property of a thorium intermetallic compound dispersion to be used as a fluid blanket is that it be pumpable. Heretofore difficulties have been encountered in avoiding dense compact crystalline forms, or grossly enlarged platelets which are up to centimeters in diameter. Neither of these forms are readily pumped.

It is therefore a principal object of the invention to provide a method of preparing a readily pumpable dispersion of thorium intermetallic compound in fine particulate form in bismuth, lead or bismuth-lead alloy.

The invention is predicated on the discovery that upon heating an alloy consisting of about 10 to 50 percent by weight of thorium the balance a magnesium metal, thereby to sublime or distill away the magnesium metal and leave a thorium sponge, and thereafter on heating the so-prepared thorium sponge in contact with a low melting metal selected from the group consisting of bismuth, lead or bismuth-lead alloy, a fine particulate, pumpable dispersion of thorium intermetallic compound is obtained.

For the purposes of the specification and claims the term "thorium intermetallic compound" refers to the intermetallic compounds of thorium with bismuth and with lead.

In carrying out the method of the invention an alloy of thorium and magnesium is provided by heating together under an inert atmosphere the requisite amounts of the metals to form an alloy consisting of about 10 to 50 percent by weight of thorium; the balance being magnesium metal.

For the purpose of the specification and claims a magnesium metal is defined as a metal selected from magnesium and magnesium alloyed with up to 5 weight percent of a volatile metal selected from the group consisting of calcium, sodium, zinc and mixtures thereof.

In accordance with the invention, an alloy of thorium and magnesium metal may also be prepared from a compound of thorium, preferably thorium fluoride. The thorium compound is heated together with an excess of molten magnesium metal under an inert atmosphere to effect the reduction of the thorium compound, the so-formed thorium alloying directly with the excess of molten magnesium metal. Intimate contact and reactivity of the relatively high melting thorium compounds with the relatively low melting magnesium metal are generally facilitated by taking up the thorium compound in a saline composition which is then admixed with molten magnesium metal. As an example, according to U.S.

## 2

Patent No. 2,678,267, thorium fluoride is admixed with NaCl and KCl to form a saline mixture which is melted and reacted with molten magnesium in the preparation of magnesium-thorium alloy.

5 In any event, the thorium alloy selected or provided by preparation thereof should contain from about 50 to 90 percent by weight of magnesium metal, more preferably 70 to 85 percent in order to form the desired porous sponge-like thorium mass during the sublimation step. 10 In order that a thorium dispersion may be formed therefrom in reasonably short times, such as 1 or 2 hours, it is essential that the residual thorium obtained in the present process have a particulate, skeletal, or cellular form in which the average shortest dimension of particle or 15 cell wall is relatively small, e.g., less than 0.1 inch. Preferably the thorium has an average shortest dimension in the range of about 0.02 to 0.05 inch.

Sublimation or distillation of the volatile light metal is carried out, broadly speaking, in a manner generally well 20 understood in the art of purifying volatile metals. The thorium alloy is placed in a suitable container, such as a molybdenum boat, which is placed in a sublimer, i.e., a horizontal furnace adapted to be evacuated and having an arrangement to collect the metal subliming or distilling 25 from the thorium alloy. The furnace is generally evacuated to a reduced pressure lower than about 0.1 mm. of Hg and heating is begun to selectively volatilize the said magnesium metal from the thorium.

Melting of the thorium once it is substantially magnesium-free is to be avoided because the formation of a 30 porous residue is thereby prevented, resulting in either a dense sponge or massive thorium, neither of which is readily dispersed in bismuth or lead. However, at the beginning of the heating period the melting of low-melting 35 magnesium-thorium intermetallic compounds is not deleterious and magnesium distills from the molten alloy. If it is desired to carry out the preparation entirely by the sublimation process, heating is commenced at a temperature at least slightly below the melting temperature of the 40 thorium alloy. In any event, the temperature is gradually increased over a period of hours to a temperature in the range of 650 to 900° C. Temperatures above 800° C. are employed to assure more complete removal of the 45 magnesium metal as well as to cause sintering of the residual thorium into a fairly coherent mass. If the thorium residue is not heated to a high enough temperature, it is crumbly and unsintered and tends to be pyrophoric on exposure to air. If the thorium intermetallic 50 compound dispersion is to be prepared in the same furnace in the absence of air, the stability in air is not important and a final temperature of about 750 to 800° C. is satisfactory. At 700 to 800° C. the sublimation process is usually completed in 5 to 10 hours, depending upon the 55 amount of alloy. Larger amounts of alloy require longer heating periods.

The resulting sponge is allowed to cool and is then dispersed in bismuth, lead or any alloy of bismuth and lead, any of which may be employed as a blanket material 60 solvent or dispersant medium in a nuclear reactor system.

If lead is employed, a dispersion of a thorium-lead intermetallic compound, such as  $\text{ThPb}_3$ , is obtained. In bismuth and most bismuth-lead alloys, a dispersion of a thorium bismuthide compound is formed, the thorium-lead compounds forming only in bismuth-lead alloy containing more than about 95 percent by weight of lead, the balance bismuth.

The dispersion process is carried out by heating one part by weight of the thorium sponge together with from 5 to 100 parts by weight of pieces of bismuth, lead or bismuth-lead alloy. The metals are placed in a suitable container such as a graphite crucible and heated in a

furnace provided with means of maintaining an inert atmosphere. At a temperature in the range of 550 to 650° C. the thorium forms thorium bismuthide or thorium-lead compound which spalls off the surface of the sponge until the conversion to intermetallic compound is completed. At temperatures above about 700° C. appreciable quantities of thorium tend to dissolve in the bismuth, lead, or bismuth-lead alloy, and on cooling the resulting thorium low-melting metal alloy very large platelets of thorium compound are precipitated. Dispersion of 10 to 20 gram quantities of thorium sponge in 100 to 200 grams of bismuth, lead, or bismuth-lead alloy is generally completed in about 45 minutes to one hour at 600° C. Larger quantities of sponge and low-melting metal require longer times.

The so-prepared dispersion of thorium intermetallic compound may be used directly as a blanket in a breeder-type nuclear reactor. Or if desired, it may first be further diluted with additional bismuth, lead, or bismuth-lead to accommodate a given reactor design.

*Example*

As an example of the process of the invention a magnesium-thorium alloy was prepared by melting together thorium and magnesium under an inert atmosphere and decanting the alloy from the dross. Forty and five-tenths (40.5) grams of the resulting alloy consisting of about 30 percent by weight of thorium, the balance magnesium, was placed in a molybdenum boat-type sublimer and the sublimer furnace was evacuated to about 0.020 mm. Hg pressure. The furnace was first brought to a temperature of 550° C. and then the temperature was brought, over the space of five hours, to 700° C. The 700° C. temperature was maintained for about seven hours to assure the complete removal of the magnesium as well as the formation of a coherent sponge weighing about 13.5 grams. The thorium sponge was placed in a graphite crucible along with .125 gram of oxide-free, 0.5 inch diameter bismuth rods. The crucible and contents were placed in an evacuable electric furnace. The furnace was purged of air and filled with an inert gas. Then the furnace was brought to and maintained at a temperature of 600° C. for one hour. During the one hour period the bismuth-thorium mixture was agitated several times. The furnace was then allowed to cool and the contents of the crucible solidified as a casting. The casting was removed from the crucible, sectioned, and examined by the metallographic method. The casting was found to consist of a finely divided dispersion in bismuth of thorium bismuthide particles which exhibited a maximum dimension of about 10 microns. Chemical examination of the casting indicated the concentration of residual magnesium was less than 200 parts per million.

We claim:

1. In the method of preparing a fine particulate dispersion of a thorium intermetallic compound selected from the group consisting of thorium-bismuth and thorium-lead intermetallic compounds, in a low-melting metal selected from the group consisting of bismuth, lead and bismuth-lead alloys, wherein a thorium sponge is prepared and heated in contact with said low-melting metal, the improved method of preparing said thorium sponge which comprises: alloying a magnesium metal selected from the group consisting of magnesium, and magnesium containing up to 5 weight percent of calcium, sodium, zinc and mixtures thereof, with thorium under an inert atmosphere, the amount of magnesium metal in the so-prepared thorium alloy being about 50 to 90 percent by weight of the alloy; and under a pressure of less than about 0.1 mm. of Hg, heating said alloy initially to a temperature of about 550° C. and thereafter gradually to a temperature in the range of 650 to 900° C., thereby

to volatilize said magnesium metal from the alloy and leave a thorium sponge.

2. In the method of preparing a fine particulate dispersion of a thorium intermetallic compound selected from the group consisting of thorium-bismuth and thorium-lead intermetallic compounds, in a low-melting metal selected from the group consisting of bismuth, lead and bismuth-lead alloys, wherein a thorium sponge is prepared and heated in contact with said low melting metal, the improved method of preparing said thorium sponge which comprises: providing an alloy consisting of thorium and a magnesium metal selected from the group consisting of magnesium, and magnesium alloyed with up to 5 weight percent of calcium, sodium, zinc, and mixtures thereof, the proportion of said magnesium metal in the alloy being about 50 to 90 percent by weight of the alloy, the balance thorium; and under a pressure of less than about 0.1 mm. of Hg, heating said alloy initially to a temperature of about 550° C. and gradually to a temperature in the range of 650 to 900° C., thereby to volatilize the magnesium metal from the alloy and leave a thorium sponge.

3. The method of preparing a fine particulate dispersion of a thorium intermetallic compound selected from the group consisting of thorium-bismuth and thorium-lead intermetallic compounds, in a low-melting metal selected from the group consisting of bismuth, lead and bismuth-lead alloys, which comprises: alloying a magnesium metal selected from the group consisting of magnesium, and magnesium alloyed with up to 5 weight percent of calcium, sodium, zinc, and mixtures thereof, with thorium under an inert atmosphere, the amount of said magnesium metal in the so-prepared alloy being about 50 to 90 percent by weight of the alloy, the balance thorium; heating said alloy under a pressure of less than about 0.1 mm. of Hg, initially to a temperature of about 550° C. and gradually to a temperature in the range of 650 to 900° C., thereby to volatilize said magnesium metal from the alloy and leave a thorium sponge having an average cellular wall thickness of less than about 0.05 inch; contacting said thorium sponge with from 5 to 100 parts by weight of said low-melting metal per part of thorium at a temperature above the melting point of the low-melting metal and below about 700° C. for a time sufficient for the thorium sponge to form an intermetallic compound of thorium and said low melting metal, thereby to precipitate said intermetallic compound in the form of solid particles having a maximum dimension of about 1 millimeter.

4. The method of preparing a fine particulate dispersion of thorium bismuthide in a low-melting metal selected from the group consisting of bismuth, and bismuth-lead alloy containing up to 90 weight percent lead, the balance bismuth, which comprises: contacting a thorium sponge-like mass having an average cellular wall thickness of less than about 0.05 inch with from 5 to 100 parts by weight of said low-melting metal per part of thorium sponge-like mass under an inert atmosphere, at a temperature above the melting point of the low-melting metal and below about 700° C. for a time sufficient for said thorium sponge-like mass to form the intermetallic compound thorium bismuthide, thereby to precipitate said intermetallic compound in the low melting metal in the form of solid particles having a maximum dimension of about 1 millimeter.

References Cited in the file of this patent

UNITED STATES PATENTS

|    |           |               |       |                |
|----|-----------|---------------|-------|----------------|
| 70 | 2,434,775 | Sosnick       | ----- | Jan. 20, 1948  |
|    | 2,910,417 | Teitel        | ----- | Oct. 27, 1959  |
|    | 2,915,445 | Bryner        | ----- | Dec. 1, 1959   |
|    | 2,952,508 | Bryner et al. | ----- | Sept. 20, 1960 |